

## UNITED STATES PATENT OFFICE

2,153,701

PROCESS FOR DYEING ANIMAL FIBERS  
WITH COMPLEX CHROMIUM COMPOUNDS  
OF AZO DYESTUFFSFritz Straub, Basel, and Hermann Schneider,  
Riehen, Switzerland, assignors to the firm of  
Society of Chemical Industry in Basle, Basel,  
SwitzerlandNo Drawing. Application February 18, 1937, Se-  
rial No. 126,520. In Switzerland February 26,  
1936

4 Claims. (Cl. 8—43)

It has been found that animal fibers, for example wool and natural silk, can be dyed with the complex chromium compounds of the azo-dyestuffs of the general formula



wherein  $\text{R}_1$  represents a naphthalene radical free of nitro groups and  $\text{R}_2$  represents a naphthalene radical containing no substituents besides the hydroxyl group, and wherein further the two hydroxyl groups stand in ortho-position to the azo-bridge, by adding the dyestuffs in portions to the dye-bath.

Complex chromium compounds of the azo-dyestuffs of the above general formula are for example the complex chromium compounds of the azo-dyestuffs from diazotized 1-amino-2-hydroxynaphthalene-4-sulfonic acid, from diazotized 2-amino-1-hydroxynaphthalene-4-sulfonic acid, as well as from diazotized chloro- or bromo-1-amino-2-hydroxynaphthalene-4-sulfonic acid and 1- or 2-hydroxynaphthalene. These complex chromium compounds may be produced according to the most different known processes. Apart from these dyestuffs there may also be used other dyestuffs, particularly such dyestuffs which are suitable for shading navy blues.

The dyestuff may be added to the dye-bath in two or more portions and at shorter or longer intervals; in many cases it is of particular advantage if the aqueous solution of the dyestuff is allowed to flow into the dye-bath during the dyeing, this flow being extended over a considerable portion of the duration of the dyeing.

In some cases it is advantageous to add to the bath a wetting agent, a dispersing agent or an emulsifying agent.

The conditions usual in dyeing animal fibres with chromium compounds of azo-dyestuffs may be observed; accordingly the animal fibers may be dyed in baths containing organic (aliphatic, aromatic or hydroaromatic) acids together with mineral acids, such as sulphuric acid, or merely in presence of sulphuric acid, in a proportion of about 5-10 per cent. of the goods to be dyed; in some cases it is also of advantage to add the acid also in portions and to begin the dyeing at about 60-90° C.

The process leads to uniform deep navy blue tints fast to rubbing, against which vegetable fibers, such as cotton and also artificial silk from regenerated cellulose or acetate artificial silk, can be reserved, whereas by dyeing with the same dyestuffs according to the customary processes there are obtained dyeings which are not uniform and are not fast to rubbing and are insufficiently reserved.

The following examples illustrate the invention, the parts being by weight.

## Example 1

100 parts of woollen piece goods are entered into a dye-bath having a temperature of 80-90° C. and composed of 3000 parts of water, 4 parts of concentrated sulphuric acid and 2 parts of the chromium compound of the azo-dyestuff of the formula



from diazotized 1-amino-2-hydroxynaphthalene-4-sulfonic acid and 2-hydroxynaphthalene. After 10 minutes the bath is heated to boiling and the material is allowed to absorb the aforesaid quantity of dyestuff for  $\frac{3}{4}$  hour.

Then further 4 parts of concentrated sulphuric acid are added and in the course of  $\frac{1}{4}$  hour there is run in a solution of 2 parts of the same chromium compound in 20 parts of water. Then the bath is kept boiling for 1-1½ hours after which the goods are washed and dried. The material is dyed excellent level navy blue tints.

## Example 2

A dye-bath is prepared with 3000 parts of water and 4 parts of concentrated sulphuric acid, and at a temperature of 90° C. 100 parts of wool are entered, moved in the bath for a short time until the material is well penetrated, and then whilst the liquor is kept in motion a solution of 3.6 parts of the chromiferous azo-dyestuff from diazotized 1-amino-2-hydroxynaphthalene-4-sulfonic acid and 2-hydroxynaphthalene in 50 parts of water is run in at 90-95° C. in the course of  $\frac{3}{4}$  hour.

hour. After an hour 4 parts of concentrated sulphuric acid are added and the bath is maintained boiling for 1-1½ hours longer; then the material is washed and dried. It is dyed deep navy blue 5 shades of excellent properties of fastness.

*Example 3*

100 parts of woollen piece goods are wetted in 10 a bath at 90° C. consisting of 2500 parts of water and 8 parts of concentrated sulphuric acid. Then a solution of 4 parts of the chromium compound of the azo-dyestuff of the formula



25 from diazotized 1-amino-2-oxynaphthalene-4-sulphonic acid and 1-oxynaphthalene in 80 parts of water is run in in the course of ¾-1 hour whilst the goods are kept in motion in the bath. The bath is then kept at the boil for 1-1½ hours longer, and the material is then washed and dried. There is obtained a level navy blue dyeing 30 properties of very good fastness.

*Example 4*

35 100 parts of woollen piece goods are entered into a dye-bath of 85-90° C. composed of 2500 parts of water and 5.8 parts of formic acid of 85 per cent. strength. In the course of 20-30 minutes there is allowed to run in a solution of 4 parts of the chromium compound of the azo-dyestuff from 40 diazotized 1-amino - 2 - oxynaphthalene - 4 - sulphonnic acid and 2-oxynaphthalene in 50 parts of water. The bath is boiled for ½ hour, 6 parts of concentrated sulphuric acid are cautiously added and boiling is continued for 1-1½ hours 45 longer; the material is then washed and dried. There are obtained navy blue shades of excellent fastness properties.

*Example 5*

50 A dye-bath of 90° C. is prepared from 3000 parts of water and 8 parts of concentrated sulphuric acid and 100 parts of loose wool are entered and moved in the bath for a short time until thoroughly penetrated. Then in the course 55 of ½-¾ hour the dyestuff solution of 5 per cent. strength, consisting of 3.2 parts of the chromiferous azo-dyestuff from diazotized 1-amino-2-oxynaphthalene-4-sulphonic acid and 2-oxynaphthalene and 0.6 part of the chromiferous 60 azo-dyestuff of the formula



70 from diazotized 1-methyl-3-amino-4-oxybenzene-6-sulphonic acid and 2-oxynaphthalene, is run in whilst the liquor is kept in motion. Simultaneously, the bath is brought slowly to the boil and kept boiling for 1-1½ hours longer; the material 75 is then washed and dried. There are obtained

reddish-navy blue shades of very good fastness properties.

*Example 6*

75 Into a dye-bath heated to 90° C. and consisting of 2400 parts of water, 8 parts of sulphuric acid of 100 per cent. strength and 8 parts crystallized sodium sulphate, 100 parts of woollen piece goods are entered and while handling the goods a dye-stuff solution of 3.6 parts of the chromium compound of the azo-dyestuff from diazotized 1-amino-2-oxynaphthalene-4-sulphonic acid and 2-oxynaphthalene made as described in Example 1 of Patent No. 1,480,640 in about 200 parts of water is allowed to run into the bath in the 10 course of ¾-1 hour.

15 The bath is then boiled, if desired with addition of water to make good that evaporated, for 1-1½ hours. The goods are then thoroughly washed with water and dried. They are dyed 20 uniform navy blue of excellent properties of fastness.

What we claim is:—

1. Process for dyeing animal fibers with complex chromium compounds of azo-dyestuffs of 25 the general formula



30 wherein  $\text{R}_1$  represents a naphthalene radical free of nitro groups and  $\text{R}_2$  represents a naphthalene radical containing no substituent besides the hydroxyl group, and wherein the two hydroxyl groups stand in ortho-position to the azo-bridge, consisting in dyeing animal fibers in a dye-bath to which the complex chromium compounds of the azo-dyestuffs are added in portions during the dyeing process.

2. Process for dyeing animal fibers with complex chromium compounds of azo-dyestuffs of the 40 general formula



45 wherein  $\text{R}_2$  represents a naphthalene radical containing no substituent besides the hydroxyl group, and wherein the hydroxyl group of the naphthalene radical  $\text{R}_2$  stands in ortho-position to the azo-bridge, consisting in dyeing animal fibers in a dye-bath to which the complex chromium compounds of the azo-dyestuffs are added in portions during the dyeing process.

3. Process for dyeing animal fibers with the 60 complex chromium compound of the azo dyestuff of the formula



65 consisting in dyeing animal fibers in a dye-bath to which the complex chromium compound of the azo-dyestuff is added in portions during the dyeing process.

4. Process for dyeing animal fibers with the 70

5

10

15

20

25

30

35

40

45

50

55

60

65

70

75

complex chromium compound of the azo-dyestuff of the formula

5



consisting in dyeing animal fibers in a dye-bath and allowing an aqueous solution of the dyestuff to run into the dye-bath during the dyeing operation, this running in being extended over a considerable period of the duration of the dyeing.

5

FRITZ STRAUB.  
HERMANN SCHNEIDER.